

## UNITED STATES PATENT OFFICE

1,922,287

CELLULOSE ESTERS AND PROCESS OF  
MAKING SAME

Robert Haller, Richen, near Basel, and Andreas Ruperti, Basel, Switzerland, assignors to firm Society of Chemical Industry in Basle, Basel, Switzerland

No Drawing. Application July 11, 1931, Serial No. 550,268, and in Switzerland February 28, 1930

10 Claims. (Cl. 260—101)

The present invention, which is an improvement in or a modification of that described in specification Serial No. 514,307, filed February 7, 1931, relates to the manufacture of new cellulose esters. It comprises the process of making these esters, as well as the esters themselves.

In the above cited specification it is shown that while the esterification of cellulose by means of acetic anhydride proceeds with difficulty in the presence of sodium acetate, the esterification of cellulose by means of aliphatic acid anhydrides occurs very easily in the presence of potassium salts of weak acids. The reaction is particularly smooth when the cellulose material, if desired after previous swelling, is first impregnated with the potassium salt, then dried and then treated with the anhydride of the aliphatic acid.

According to the present invention cellulose material can be esterified in high degree and easily by means of an aliphatic acid anhydride in presence of a sodium salt of a weak acid, if, instead of adding the sodium salt to the esterifying bath, the procedure recommended in the aforesaid specification is followed. It is necessary to operate under conditions imparting a somewhat energetic reaction. Among other conditions, the esterification advantageously proceeds at a temperature not too low.

In the present invention the same weak acids as named in application Serial No. 514,307 may be used, such as acetic acid, carbonic acid, propionic acid, butyric acid, stearic acid, sulfuric acid, etc.

As acid anhydrides the same anhydrides are also coming into consideration which are stated in application Serial No. 514,307, such as the anhydride of acetic acid, propionic acid, butyric acid, valeric acid, isovaleric acid, isobutyric acid, monochloracetic acid, etc.

The following examples illustrate the invention, the parts being by weight:—

## Example 1

100 parts of cotton are immersed for 1 hour in 1,000 parts of mercerizing caustic soda solution, then removed from the bath, centrifuged and thoroughly washed with water and again centrifuged; without drying the cotton is then immersed in 1000 parts of a saturated aqueous solution of sodium acetate. After 1 hour the material is removed from the liquor, centrifuged, dried and heated in acetic anhydride to boiling for 1 hour. The liquor is run off, while hot, and regenerated. The cellulose material, if desired after the separation of the adherent liquid by

drying it in a vacuum, is washed with water and dried.

There are obtained 145 parts of an ester having the original fibrous structure, and containing approximately 2 acetyl-groups per  $C_6H_{10}O_5$  unit. It is insoluble in organic solvents and is well suited for being worked up into soluble esters.

## Example 2

100 parts of viscose artificial silk are immersed in 1000 parts of a saturated aqueous solution of sodium acetate. After an hour the silk is removed from the bath, dried and heated for 1 hour to boiling in a solution of 250 parts of acetic anhydride in 800 parts of xylene. After cooling, the silk material is freed from adhering liquor by centrifuging and drying in a vacuum. It is then washed with water and dried. There are obtained 130–135 parts of an ester silk having the properties similar to those described for the product obtained with use of potassium acetate in specification Serial No. 514,307 of 1931.

The esterification of cellulose artificial silk described in this example can obviously be conducted at any suitable stage of the manufacture. It may be applied even to the finished web or to dyed material, as has been explained in specification Serial No. 514,307.

## Example 3

100 parts of wood pulp are soaked overnight in mercerizing caustic soda solution (18 per cent. strength), then pressed until the weight is three times that of the cellulose material, disintegrated in the Werner-Pfleiderer apparatus and treated with a quantity of acetic acid equivalent to the alkali present, so as to neutralize the latter. The material, if necessary with aid of a vacuum, is dried in a drying chest, and acetylated as described in Example 1. The product is similar to that obtained according to Example 1.

What we claim is:—

1. A process for esterifying cellulose whilst maintaining its structure, which consists in impregnating the cellulose with a solution of a sodium salt of a weak acid, drying and esterifying the material in the heat with an aliphatic acid anhydride in the absence of an acid catalyst.

2. A process for esterifying cellulose whilst maintaining its structure, which consists in impregnating the cellulose with a solution of a sodium salt of a weak aliphatic acid, drying and

65

70

75

80

85

90

95

100

105

110

esterifying the material in the heat with an aliphatic acid anhydride in the absence of an acid catalyst.

3. A process for esterifying textile materials consisting of cellulose whilst maintaining their structure, which consists in impregnating the material with a solution of a sodium salt of a weak aliphatic acid, drying and esterifying it in the heat with an aliphatic acid anhydride in the absence of an acid catalyst.

4. A process for esterifying textile materials consisting of cellulose whilst maintaining their structure, which consists in impregnating the swelled material with a solution of sodium acetate, drying and esterifying it in the heat with acetic acid anhydride in the absence of an acid catalyst.

5. A process for esterifying regenerated cellulose whilst maintaining its structure, which consists in impregnating regenerated cellulose with a solution of a sodium salt of a weak acid, drying and esterifying the material in the heat with an aliphatic acid anhydride in the absence of an acid catalyst.

6. A process for esterifying regenerated cellulose whilst maintaining its structure, which consists in impregnating regenerated cellulose with a solution of sodium acetate, drying and esterifying the material in the heat with acetic acid anhydride in the absence of an acid catalyst.

7. A cellulose ester which is obtained by esterifying cellulose impregnated with a solution of a sodium salt of a weak acid with an aliphatic acid anhydride in the absence of an acid catalyst, the esterification being conducted in the heat, which product is insoluble in chloroform and acetone and constitutes an ester of non-degraded cellulose.

sodium salt of a weak acid with an aliphatic acid anhydride in the absence of an acid catalyst, the esterification being conducted in the heat, which product is insoluble in chloroform and acetone and constitutes an ester of non-degraded cellulose.

8. A cellulose ester which is obtained by esterifying cellulose impregnated with a solution of a sodium salt of a weak aliphatic acid with an aliphatic acid anhydride in the absence of an acid catalyst, the esterification being conducted in the heat, which product is insoluble in chloroform and acetone and constitutes an ester of non-degraded cellulose.

9. A cellulose ester which is obtained by esterifying regenerated cellulose impregnated with a solution of a sodium salt of a weak acid with an aliphatic acid anhydride in the absence of an acid catalyst, the esterification being conducted in the heat, which product is insoluble in chloroform and acetone and constitutes an ester of non-degraded cellulose.

10. A cellulose ester which is obtained by esterifying regenerated cellulose impregnated with a solution of sodium acetate with acetic acid anhydride in the absence of an acid catalyst, the esterification being conducted in the heat, which product is insoluble in chloroform and acetone and constitutes an ester of non-degraded cellulose.

ROBERT HALLER.  
ANDREAS RUPERTI.

35

110

40

115

45

120

50

125

55

130

60

135

65

140

70

145

75

150